

## UNITED STATES PATENT OFFICE

2,536,989

DIAZOTYPE LAYERS CONTAINING RESOR-  
CINOL DERIVATIVES

William H. von Glahn, Loudonville, and Lester N. Stanley, Delmar, N. Y., assignors to General Aniline & Film Corporation, New York, N. Y., a corporation of Delaware

No Drawing. Application January 20, 1948,  
Serial No. 3,326

8 Claims. (Cl. 95—6)

1

This invention relates to a diazotype process and photoprinting materials, and more particularly to the use of certain azo coupling components in the light sensitive layer or in developers for the diazotype image.

In the reproduction of mechanical drawings, printed material, pictures or other originals to be copied, it is of particular advantage in many cases to first make an intermediate print or "transition" print on a transparent diazotype copying material by exposing a transparent sensitized diazotype material to actinic rays by either the printing-through or reflex process and then developing the diazotype material. The image thus produced on the intermediate or transition diazotype print can then be used for the reproduction of further diazotype prints in the usual manner, of high contrast. This method is particularly useful when it is desired to make a number of reproductions from a frail or valuable original which would be adversely affected, if not destroyed, in the repeated exposures necessary to make a large number of copies.

The efficiency of the process involving the production of a transition or intermediate print depends upon the opacity of the azo dye image produced upon such intermediate or such transition print to ultraviolet light and upon the transparency of the background portions thereof. It depends also upon the visual density of the image produced on the intermediate or transition print, since images of poor visual density, such as yellow on a white or transparent background, while having the desired degree of opacity to ultraviolet light, nevertheless, have the disadvantage of rendering difficult the detection of flaws in the intermediate image, and it is often necessary to make a contrasting print from the transition print before such flaws can be detected.

Prints of a deep color having a good visual density can be obtained from diazotypes including such azo components as phloroglucinol, but despite the density of the color constituting the image, its actinic opacity or photographic density is insufficient to reproduce the image satisfactorily in diazotype copies made therefrom. The azo coupling component used for the production of such images on prints which are to be used as intermediate or transition copies must be such as to produce, upon coupling with the diazo compound employed, a yellow to brown azo dye which will sufficiently absorb ultraviolet light to prevent decomposition by light of the diazo compound in the areas to be reproduced from the intermediate or transition copies.

2

Coupling components such as resorcinol have been employed heretofore in diazotype transition print light sensitive layers for the production of color images having the desired light absorption characteristics for transition printing. While resorcinol will produce the image on the transition print in azo dye colorations having good opacity to ultraviolet light and having sufficient visual density to assure detection of printing flaws, the pre-coupling stability of the diazotype layer is not sufficient to permit prolonged storage before use. It has been found that carriers, such as transparentized paper or film, having thereon a light sensitive layer composed of the usual diazo components and resorcinol gradually develop a discoloration prior to use, which discoloration is produced by premature coupling of the resorcinol and the diazo component. This discoloration will, of course, be retained by the transition print and impairs the capacity of the background areas to transmit actinic light. Consequently, the light sensitive diazo components in the diazotype media employed for copying from the transition print will not be efficiently decomposed in the background areas. This same discoloration, therefore, will be reproduced in the final copies, diminishing the contrast between the background and the image.

In addition, the colorations produced with resorcinol are in many cases not fast to light, and tend to fade over a period of time, particularly when exposed to prolonged or repeated actinic radiation used in making final copies from the transition prints. Furthermore, colorations thus produced often tend to offset; for example, they rub off when the transition copy is passed over hot rollers in the printing machine. When resorcinol is employed for the development of one-component diazotype layers, wherein the coupling component is applied in an aqueous developing solution to the previously exposed diazotype material, or when a two-component layer containing resorcinol as the coupling component is developed by a wet or semi-wet process in which an aqueous alkaline solution is applied to the exposed layer, the coloration produced tends to bleed by reason of its comparative solubility in the aqueous developing liquid.

It has now been found that a new class of azo coupling components, not heretofore used in diazotype reproduction, can be employed in a light sensitive layer together with a suitable light sensitive diazo compound, or as a developer for a one-component diazotype layer, to form an image in a sepia color of high actinic opacity and good

visual density, while at the same time avoiding the difficulties mentioned above which are encountered by similar use of resorcinol. The class of compounds employed as azo coupling components in accordance with this invention are carbonic ester derivatives of resorcinol which can be prepared by reacting resorcinol with phosgene in the presence of a suitable HCl acceptor or reaction medium, such as pyridine, dimethyl aniline, quinoline or other tertiary nitrogen bases. Preparation of such compounds is disclosed by Einhorn in Liebeg's Annalen 300, page 152.

The reaction of resorcinol with phosgene under the aforesaid conditions apparently results in the formation of carbonic acid ester derivatives of resorcinol of which the exact constitution is in doubt, but apparently varying according to the proportions of the inter-reacting reagents from di-resorcylic carbonate (resulting from reaction of 2 moles of resorcinol with 1 mol of phosgene) to polymeric resorcinol carbonates of molecular size which increases as the proportion of phosgene reacting with the resorcinol approaches an equimolecular amount. The probable general formula for the carbonic ester derivatives of resorcinol of this invention is as follows:



wherein  $n$  is an integer of the series of 0, 1, 2, 3 . . . All of the compositions or mixtures formed by the aforesaid reaction can be used as coupling components in diazotype compositions and processes in accordance with this invention.

While it is not desired to limit the invention to any theory, it is believed that the aforesaid carbonic ester derivatives of resorcinol, particularly those of relatively complex structure, are incapable of coupling per se with light sensitive diazo components, and hence, when used in a two-component diazotype layer, the latter is stable to premature coupling, even upon prolonged storage. However, under the alkaline conditions prevailing during development, the aforesaid resorcinol derivatives are decomposed to form less complex compounds adapted to couple with the diazo component. Regardless of the correctness of this theory, it has been found that when the resorcinol derivatives of this invention are employed together with a light sensitive diazo compound in a two-component diazotype layer, the product obtained possesses a high degree of stability against premature coupling under the usual conditions of temperature and humidity to which it is subjected during prolonged storage, as well as under accelerated aging tests which simulate the effect of prolonged storage.

Thus, it is possible in accordance with the invention, to make transition prints having a colorless background of excellent actinic transparency from two-component diazotype materials which include the resorcinol derivatives of this invention as coupling components, even after prolonged storage such as may be required for commercial distribution of the material. In this respect, the resulting transition prints are vastly superior to those obtained with diazotype materials containing resorcinol itself as the coupling component. The image produced with materials of this invention has equal or better covering power and opacity to ultraviolet light, superior fastness to light and washing, better visual density, and greatly improved resistance to offsetting as com-

pared with transition prints produced with resorcinol. The transition prints produced in accordance with the invention are therefore highly advantageous for the production of large numbers of copies.

In the preparation of diazotype layers or materials for use in making intermediate or transition copies in accordance with this invention, a transparent base such as transparentized paper, a film 10 of transparent plastic material such as regenerated cellulose or an organic derivative of cellulose (cellulose ethers and esters such as ethyl cellulose or cellulose acetate) can be used. The base is coated or impregnated with a sensitizing composition in any manner known to the art, particularly by applying thereto a solution containing the light sensitive diazo compound together with the other ingredients ordinarily used in diazotype sensitizing compositions such as metal salts, stabilizers, anti-oxidants, humectants and the like. The solvent medium employed is preferably compounded to penetrate or impregnate the base material and ordinarily contains a substantial proportion of water to insure solution of the sensitizing components therein. In preparing two-component diazotype material in accordance with this invention, a carbonic ester derivative of resorcinol of the type described above is incorporated in the sensitizing composition, or can be applied separately (e. g., by applying it in a separate solution or by rubbing it in powdered form on the surface of the carrier).

As light sensitive diazo components, we prefer to use those which are derived from p-diamines of the benzene series, particularly those in which at least one of the hydrogens of one of the amino groups is substituted by such groups as alkyl, alkoxyalkyl, aryl, aralkyl, alkylol, cycloaliphatic and heterocyclic groups. However, other diazo components have also been found suitable, such as diazo anhydrides of amino naphthols. These diazo compounds can be used in the form of stabilized derivatives such as the zinc, cadmium or tin chloride double salts, fluoroborates, or alkyl or aryl sulfonate complexes. Examples of amines from which suitable light sensitive diazo compounds are derived include p-amino-N-(2'-hydroxyethyl)-N-methyl-amino-benzene, p-amino-diphenylamine, mono-ethylamino-2-(or -3-) 40 methyl - 4 - aminobenzene, 1 - N - ethyl - N - (2'-hydroxyethyl) -amino-3-methyl-4-aminobenzene, 1-N, N-diethylamino-3-ethoxy-4-aminobenzene, 1-N-benzoylamino-2, 5-diethoxy-(or dimethoxy)- 4-aminobenzene, 1-N, N-diethylamino-4-amino-benzene, 1-N, N-di-(2'-hydroxyethyl)-amino-3-chloro-4-aminobenzene, 1-N-benzyl-N-ethylamino-4-aminobenzene, 1-N, N-dimethylamino-4-aminobenzene, 1-ethylamino-4-aminobenzene, 1-N-ethyl - N - (2' - hydroxyethyl) -amino-4-amino-benzene, p-phenylene diamine, 1 - N - di(2' - hydroxyethyl) -amino-4-aminobenzene, and 2, 5-diethoxy-4-(p-ethoxyphenyl) aniline.

The light sensitive layers can be sensitized by any of the various methods employed in diazotype processes. For example, the carbonic ester derivatives of resorcinol described above can be applied to the transparent or semi-transparent base or carrier in a coating solution, together with a stabilized diazo compound, or the aforesaid coupling components can be rubbed on the surface to be sensitized in powdered form before or after application of the diazo compound. In a one-component system, the sensitive layer is formed by applying the light sensitive diazo component without the coupling component to a transparent

on semi-transparent carrier, and in this case a coupling component of the type described above and prepared in accordance with this invention is incorporated in the developing solution which is applied to the diazotype layer after exposure to light in accordance with the pre-determined original design or pattern to be reproduced.

In any of the foregoing methods, the coating solution applied to the carrier surface can be sprayed and dried, or applied by a dip method as in the case of acetate film, or by drawing the surface to be sensitized through a trough and removing the excess coating solution by means of a doctor blade. The following examples, wherein parts are by weight unless otherwise specified, illustrate but do not limit the invention.

*Example 1*

Transparentized paper was coated with a solution containing the following ingredients and made up with water to a volume of 100 cc.:

3.8 g. of carbonic ester derivative of resorcinol, prepared by reaction of 1 mol of resorcinol with 1 mol of phosgene  
 4.0 g. of N-(2'-hydroxyethyl)-N-methylaniline-p-diazo zinc chloride double salt  
 5 cc. isopropanol  
 5 cc. ethylene glycol  
 8 g. citric acid  
 4 g. thiourea  
 0.5 g. saponin

The paper coated with the foregoing composition was dried and then submitted to an accelerated aging test, together with a sample of control material coated with a similar sensitizing composition, except that it contained resorcinol instead of the carbonic ester derivative of resorcinol as the azo coupling component. The sensitized materials were exposed to light under an original, and the image developed by treatment with ammonia fumes. The copy produced from the material sensitized in accordance with the invention yielded a clear sharp image of the original with colorless background areas, whereas the control sample prepared with resorcinol showed considerable discoloration in the background areas. The pattern of the original was reproduced on the material in accordance with the invention in a darker and less reddish sepia shade of excellent visual density which possessed greater opacity to ultraviolet light, superior fastness to light and washing, and greater resistance to offsetting than the image obtained on the resorcinol-containing control material. Further prints were obtained on ordinary diazotype photoprinting material by employing the copies produced with the transition printing material of this example as the original, the resulting copies having excellent line density and sharpness, and no background discoloration.

*Example 2*

Transparentized paper was coated with a solution made up with water to a volume of 100 cc., containing the following ingredients:

4 g. of a carbonic ester derivative of resorcinol, prepared by reaction of 2 mols of resorcinol with 1 mol of phosgene  
 4 g. of N-(2'-hydroxyethyl)-N-methylaniline-p-diazo zinc chloride double salt  
 5 cc. isopropanol  
 5 cc. ethylene glycol  
 8 g. citric acid  
 4 g. thiourea  
 0.5 g. saponin

The sensitized material thus obtained was employed in the manner described in the preceding example for the preparation of transition prints, and likewise tested to compare it with material prepared in similar manner but containing resorcinol instead of the aforesaid carbonic ester derivative of resorcinol. Superior results were obtained similar to those of Example 1.

*Example 3*

Transparentized paper was coated with a solution made up to a volume of 100 cc. with water, containing the following ingredients:

3.4 g. of a carbonic ester derivative of resorcinol, prepared by reacting 1 mol of resorcinol with 1 mol of phosgene  
 3.6 g. of N-ethyl-aniline-p-diazo zinc chloride double salt  
 0.8 g. citric acid  
 1.5 cc. phosphoric acid  
 5.0 cc. isopropanol  
 4.0 g. thiourea

Upon use of the resulting sensitized material for the preparation of transition prints and subsequent use of these prints for making additional copies, results were obtained showing advantages similar to those obtained in the preceding examples.

Similar results are obtained when 3.9 g. of N,N-diethylaniline-p-diazo zinc chloride double salt are substituted for the N-ethyl-aniline-p-diazo compound in the sensitizing solution of this example.

*Example 4*

Transparentized paper was coated with a solution, made up to a volume of 100 cc. with water, containing the following ingredients:

4.0 g. of a carbonic ester derivative of resorcinol, prepared by reacting 2 mols of resorcinol with 1 mol of phosgene  
 4.0 g. N-ethyl-o-toluidine-p-diazo zinc chloride double salt  
 5.0 cc. isopropanol  
 5.0 cc. ethylene glycol  
 8.0 g. citric acid  
 4.0 g. thiourea  
 0.5 g. saponin

Transition prints prepared with the sensitized material obtained on drying were characterized by advantages and properties similar to those of the prints obtained in the preceding examples.

As indicated by the comparative accelerated aging tests, the diazotype transition print materials of each of the foregoing examples possess excellent stability against premature coupling during prolonged storage under average atmospheric conditions and are superior in this respect to similar materials in which resorcinol is used as the coupling component.

Instead of developing the images in the foregoing examples by the dry process involving treatment with ammonia vapor, an aqueous alkaline solution such as a solution of an alkali metal carbonate or tertiary phosphate (e. g., a 5-20% aqueous sodium carbonate solution) can be applied in a wet or semi-wet development step to the sensitized materials after they have been exposed to light under an original to be reproduced. The prints prepared in this manner have clear sharply defined images accurately reproducing the original; whereas, when resorcinol is used instead of the carbonic ester derivatives of the invention, the images tend to become blurred

by reason of the comparatively water-sensitive nature of the coloration produced.

One-component diazotype transition print material can be made in the same manner as disclosed in the examples, except that the carbonic ester derivatives of resorcinol are omitted in preparing the sensitizing compositions, and are included instead in an aqueous alkaline developing solution which is applied to the prints after exposure to light in accordance with a predetermined original design or pattern. Such solutions contain for example alkaline reacting salts such as alkali metal carbonates or tertiary phosphates, and the carbonic ester derivative of resorcinol, the latter being employed, for example, in a concentration of 1 to 10%. The alkaline salts, e. g., sodium carbonate, can be used, for example, in a concentration of 5 to 20%. As in wet development of two-component systems, sharp images are thus obtained, which are superior in this respect to prints similarly obtained by use of resorcinol as the developer. In other respects, the prints obtained in wet development of one- or two-component layers in accordance with the invention have the same advantages as described in the examples.

Instead of transparentized paper, films, e. g., of regenerated cellulose or of organic derivatives of cellulose, such as cellulose acetate or ethyl cellulose, can be used as the carrier and sensitized with compositions similar to those in the examples. Ordinary paper or other opaque carriers can be used where transparency is not desired in the copies produced.

Other variations and modifications, which will be obvious to those skilled in the art, can be made in the compositions, materials and processes hereinbefore described, without departing from the scope or nature of the invention.

We claim:

1. In the process of preparing diazotype copies, the step which comprises reacting the residual light sensitive diazo compound contained in a light sensitive diazotype layer after exposure thereof to light in a pre-determined pattern, with a carbonic ester which is a reaction product of 1 mol of phosgene with 1 to 2 mols of resorcinol in the presence of an alkaline reagent.

2. In the process of preparing diazotype transition copies involving exposure of a transparent carrier, having thereon a sensitized layer containing a light sensitive diazo compound, to light in a pre-determined pattern, the improvement which comprises developing the image thereby formed by reaction of the residual diazo compound with a carbonic ester which is a reaction

product of 1 mol of phosgene with 1 to 2 mols of resorcinol in the presence of an alkaline reagent.

3. A light sensitive diazotype layer on a suitable base, containing a light sensitive diazo compound and a carbonic ester which is a reaction product of 1 mol of phosgene with 1 to 2 mols of resorcinol.

4. Diazotype phototyping material for transition copies comprising a transparent carrier having thereon a light sensitive layer comprising a light sensitive diazo compound and a carbonic ester which is a reaction product of 1 mol of phosgene with 1 to 2 mols of resorcinol.

5. Diazotype phototyping material comprising a carrier having thereon a light sensitive layer containing a diazotized p-diamine of the benzene series and a carbonic ester which is a reaction product of 1 mol of phosgene with 1 to 2 mols of resorcinol.

10 6. Diazotype phototyping material for transition copies comprising a transparent carrier having thereon a light sensitive layer containing a diazo compound of 1-mono-ethylamino-2-methyl-4-aminobenzene, and a carbonic ester which is a reaction product of 1 mol of phosgene with 1 to 2 mols of resorcinol.

15 7. Diazotype phototyping material for transition copies comprising a transparent carrier having thereon a light sensitive layer containing a diazo compound of 1-N,N-diethylamino-4-amino-benzene and a carbonic ester which is a reaction product of 1 mol of phosgene with 1 to 2 mols of resorcinol.

20 8. Diazotype phototyping material for transition copies comprising a transparent carrier having thereon a light sensitive layer containing a diazo compound of N-2'-hydroxyethyl)-N-methylamino-p-aminobenzene and a carbonic ester which is a reaction product of 1 mol of phosgene with 1 to 2 mols of resorcinol.

25 9. Diazotype phototyping material for transition copies comprising a transparent carrier having thereon a light sensitive layer containing a diazo compound of 1-N,N-diethylamino-4-amino-

30 benzene and a carbonic ester which is a reaction product of 1 mol of phosgene with 1 to 2 mols of resorcinol.

35 10. Diazotype phototyping material for transition copies comprising a transparent carrier having thereon a light sensitive layer containing a diazo compound of 1-N,N-diethylamino-4-amino-

30 benzene and a carbonic ester which is a reaction product of 1 mol of phosgene with 1 to 2 mols of resorcinol.

WILLIAM H. VON GLAHN.  
LESTER N. STANLEY.

#### REFERENCES CITED

45 The following references are of record in the file of this patent:

#### UNITED STATES PATENTS

| Number       | Name             | Date          |
|--------------|------------------|---------------|
| 50 2,246,425 | von Poser et al. | Jan. 17, 1941 |
| 2,334,495    | Kendall          | Nov. 16, 1943 |
| 2,437,863    | von Glahn et al. | Mar. 16, 1948 |

#### FOREIGN PATENTS

| Number     | Country | Date          |
|------------|---------|---------------|
| 55 836,144 | France  | Oct. 10, 1938 |